

## UNITED STATES PATENT OFFICE

PAUL CHRISTIAAN VAN DER WILLIGEN, OF KROMMENIE, NETHERLANDS, ASSIGNOR OF ONE-HALF TO N. V. NEDERLANDSCHE LINOLEUMFABRIEK, OF KROMMENIE, NETHERLANDS, A DUTCH LIMITED COMPANY

## PROCESS FOR THE PRODUCTION OF FLEXIBLE FLOOR-, WALL- AND LIKE COVERS

No Drawing. Application filed November 23, 1928, Serial No. 321,518, and in the Netherlands December 8, 1927.

This invention relates to a process for the production of flexible floor-, wall- and like covers, which process differs essentially from the usual way of manufacturing.

5 According to the known processes the manufacture of these covers or of linoleum takes always place by mixing the composing constituents in numerous and expensive mixers and kneading machines. According to 10 this invention these machines becomes superfluous by bringing the composing constituents into colloid suspension, respectively colloid emulsion and preferably using water or aqueous solutions as dispersing means. Then the 15 colloid suspension, respectively colloid emulsions are mixed, after which the system is coagulated either by adding electrolytes, or by means of the electric current or otherw'se. It will be manifest, that the substances, which 20 are dispersed in water, must be as finely divided as possible. Though water is preferred by virtue of its cheapness, the process of the invention may also be carried out by means of other solvents.

25 Whereas in the manufacture of linoleum the mixing of linoxyne and the fillers and colouring substances is effected in a long way and costs much energy, the mixing of colloid solutions immediately gives a substantially 30 perfect mixture of the dispersed substances and the coagulation can be effected in such a way, that said intensive mixture rests maintained or is even improved. When the aqueous solution has been removed, the coagulated 35 mass may be used for manufacturing floor- or similar covers.

According to a further feature of this invention, the usually employed binding means for linoleum, viz. oxidized oils or linoxyne 40 may be substituted by other hydrophobe binding means, e. g. rubber or asphalt.

In general the starting materials may be considered to be colloid suspensions, respectively colloid emulsions of substances, which 45 in the coagulated state do not swell with or dissolve in water and which form a plastic, elastic mass. Particularly suitable are colloid emulsions of oils, respectively oxidized oils or polymerized oils or latex and asphaltic emulsions, or mixtures of these emulsions.

When using colloid emulsions of oils, the mass, consisting of lumps and grains, obtained after the removal of the greater part of the water, may be oxidized by means of air or otherwise. By reason of the great surface 55 the oxidation occurs in a short time in contradistinction to the oxidation of the liquid linseed oil in the linoleum manufacture according to the Walton process, which costs much time, since the surface of the linseed oil is 60 flat.

When using latex, a vulcanizer must be added, which is in colloid solution before the coagulation. Substances in crystalloid solution are generally of no use, since these substances only pass for a small part into the mass. The same applies to the accelerator and the anti-ager to be added and occasionally for the softening agents, which are often employed in rubber manufacture, 70

When using colloid asphaltic emulsions it is to be recommended to add a softening agent, for which purpose different oils (e. g. linseed oil or castor oil, etc.) in emulsified state may be used. 75

In the linoleum manufacture cork or wood-meal is much employed as elastic filler. These materials can be easily brought in aqueous colloid suspension, provided they are in a very finely divided state. 80

This may be effected by vigorously stirring these very fine materials in a solution of soap, joiner's glue or an analogous emulsifying agent. However this invention is not at all limited to the particular method of preparing the colloid suspensions or emulsions. As known one can make colloid aqueous suspensions from most of the paints or colouring substances and fillers as e. g.  $\text{BaSO}_4$ ,  $\text{CaCO}_3$ ,  $\text{ZnO}$ , lithopone, china-clay, etc. provided the starting material consists of very fine particles or arises in this form in the reaction mixture. 85

As coagulating electrolytes may be used e. g. solutions of salts, as  $\text{BaCl}_2$ , alum or acids, as  $\text{HCl}$  or acetic acid. Alternatively the electric current may effect the coagulation. 95

The coagulated mass may be freed from most of the water, e. g. by means of decanting 100

or filtering. The remaining water is removed before or during the making into the floor- or other cover, which e. g. may be effected by pressing.

5 The advantage of executing the manufacture in an aqueous medium is here also apparent, since all soluble substances, which were eventually present in the starting materials or are added during the manufacture, 10 are removed when the water is separated so that a floor cover is obtained, which only consists of material, which is not soluble in water. The feature that the covers according to this invention are not acted upon by 15 water is a very important property for floor-covers. When starting from glue, gelatine, starch, paper-fibres, etc. this property can not at all or only incompletely be obtained, no matter in which way the tanning has been 20 performed.

The invention is illustrated by the following example, but is not limited to the quantities or materials specified herein.

Example.—

25 50 liters of a colloid emulsion (containing 25% of linoxyne and 5% of resin) are mixed with 100 liters of an aqueous colloid suspension of 10 kg of corkmeal, 10 kg of china-clay and 10 kg of ochre with 0,5 kg of joiner's glue 30 as emulsifying agent. The emulsion of linoxyne and resin may be prepared by dissolving these substances in a solvent, e. g. acetic acid and pouring this solution in water.

35 However any method of preparing the emulsion is suitable for this purpose and the invention is not limited to this particular method of preparing same.

40 When the colloid emulsion and suspensions are mixed, the whole system is coagulated. 45 During all these operations the mass is quickly mechanically stirred. Then the greater part of water is removed by filtration and the mass is dried and made in a press or otherwise into floor cover with a thickness of a few 50 millimeters.

55 In the case of rubber latex colloid sulfur may be added in such a quantity, that the proportion of rubber to sulfur is approximately 100:5. Moreover a small quantity of an 60 accelerator e. g. diphenylthiourea in a colloid solution (obtained e. g. by pouring an alcoholic solution in water) may be added. The manufacture takes place in the same way as described with reference to the process with 65 linoxyne, but the final product may be heated in order to finish the vulcanization.

70 The floor covers or similar covers, produced according to this invention excel by their elasticity, flexibility, and waterproof 75 quality and moreover by a great tensile strength. By virtue of this feature the use of expensive textile fabrics may be omitted in these covers in several cases.

80 As a result of this feature considerable expenses are avoided compared to linoleum.

Moreover the whole process lasts a very short time only and requires little power, so that a greater economy is obtained yet.

Having now described my invention, what I claim as new and desire to secure by Letters Patent is:

1. A method of manufacturing a composition covering material which comprises, mixing colloidal emulsions of latex, asphalt and linoxyne with coloring and filling matter in substantially colloidal suspended form, and then coagulating the mixture. 75

2. A method of manufacturing a composition covering material which comprises mixing colloidal emulsions of latex, asphalt and linoxyne with coloring and filling matter in substantially colloidal suspended form, and then coagulating the mixture electrolytically. 80

3. A method of manufacturing linoleum, which comprises mixing a colloidal suspension of linoxyne with a substantially colloidal suspension of filling and coloring substances, and then coagulating the mixture, and working up the coagulated mass into a flat layer. 85

In testimony whereof I have signed my name to this specification.

PAUL CHRISTIAAN van der WILLIGEN.

95

100

105

110

115

120

125

130